

## [54] DIRECT-POSITIVE SILVER HALIDE PHOTOGRAPHIC LIGHT-SENSITIVE MATERIAL AND METHOD OF PROCESSING IT

[75] Inventors: Tomomi Yoshizawa; Keiji Ogi, both of Tokyo; Yasuo Tosaka; Kazuya Kuramoto, both of Odawara; Yoshiyuki Nonaka, Odawara, all of Japan

[73] Assignee: Konica Corporation, Tokyo, Japan

[21] Appl. No.: 288,022

[22] Filed: Dec. 21, 1988

## [30] Foreign Application Priority Data

Dec. 23, 1987 [JP] Japan ..... 62-326066  
Feb. 29, 1988 [JP] Japan ..... 63-47179

[51] Int. Cl.<sup>5</sup> ..... G03C 7/38; G03C 7/30

[52] U.S. Cl. ..... 430/378; 430/505;  
430/506; 430/547; 430/558; 430/567

[58] Field of Search ..... 430/547, 558 R, 378,  
430/940, 567, 506, 505

## [56] References Cited

## U.S. PATENT DOCUMENTS

4,444,865 4/1984 Silverman et al. ..... 430/940  
4,749,644 6/1988 Tosaka et al. ..... 430/547  
4,801,520 1/1989 Inoue et al. ..... 430/547  
4,830,956 5/1989 Waki ..... 430/558

## FOREIGN PATENT DOCUMENTS

230997 8/1987 European Pat. Off.  
1810464 9/1969 Fed. Rep. of Germany

## OTHER PUBLICATIONS

Patent Abstracts of Japan, vol. 11, No. 233 (P-600)  
[2680], 7/30/87, JPA 62-44731.

Primary Examiner—Richard L. Schilling  
Attorney, Agent, or Firm—Jordan B. Bierman

## [57] ABSTRACT

A direct positive type silver halide color photographic material and an image forming method are disclosed. A green sensitive emulsion layer of the photographic material comprises silver halide grains having at least two peaks on the size distribution curve thereof and the grain size corresponding to the smallest grain size peak among the peaks is not more than 0.3  $\mu$ m and a magenta coupler represented by the following Formula (M-I);



Formula (M-I)

wherein Z is a group of non-metal atoms necessary to complete a nitrogen-containing heterocyclic ring; X is a hydrogen atom or a split-off group and R is a substituent. The photographic material is developed with a color development in the presence of a fogging agent to directly form the positive image after imagewise exposure to light. Thus obtained image is improved in a increased maximum density, lowered minimum density and wider exposure latitude. Stability of gradation with respect to variation of development conditions is also improved.

51 Claims, No Drawings

**DIRECT-POSITIVE SILVER HALIDE  
PHOTOGRAPHIC LIGHT-SENSITIVE MATERIAL  
AND METHOD OF PROCESSING IT**

**FIELD OF THE INVENTION**

The present invention relates to a direct-positive silver halide photographic light-sensitive material that can obtain positive images by subjecting it to developing in the presence of a fogging agent, and a method of processing it. More particularly it is concerned with a direct-positive silver halide photographic light-sensitive material that can have a sufficiently high maximum density, yet having a sufficiently low minimum density, can have a good image quality, also can have a broad gradient, and further can be processed with a stable balance of the gradation at the toe against variations of processing conditions, and a method of processing the same.

**BACKGROUND OF THE INVENTION**

Mainly two types are hitherto known as methods of forming a direct-positive image. One of them is a method in which fog nuclei are previously formed in silver halide grains, and the fog nuclei are imagewise destroyed by solarization, Herschel effect or the like, and the remaining fog nuclei are developed to form a positive image. The other type is a method in which an internal latent image silver halide emulsion not previously fogged is used, which is subjected to fogging treatment (development nucleus formation treatment) after imagewise exposure and then surface development is carried out, or the surface development is carried out while applying fogging treatment (development nucleus formation treatment) after imagewise exposure, to form a positive image.

Of the two methods for the formation of positive image as described above, the latter type method can achieve in general a higher speed than the former type method, thus being suited to the application in which a high speed is required.

In the present technical field, various techniques have been hitherto known. For example, methods are known which are described in U.S. Pat. Nos. 2,592,250, 2,466,957, 2,497,875, 2,588,982, 3,762, 266, 3,761,276 and 3,796,577, and British Pat. No. 1,151,363.

The above methods for the fogging treatment (development nucleus formation treatment) may be carried out either by giving the whole surface exposure or by chemical procedures using a fogging agent, also by using a strong developing solution, or further by heating or the like.

Employment of these known techniques enables preparation of photographic light-sensitive materials that form positive images, but more improvement in photographic performance and solution of problems in manufacture have been sought in order to bring these photographic light-sensitive materials to be applicable in every photographic field.

In the present technical field, it is commonly known to prepare a direct-positive silver halide photographic light-sensitive material with use of two or more kinds of internal latent image emulsions. For example, U.S. Pat. No. 4,035,185 discloses that core/shell emulsions with varied degrees of internal chemical sensitization are mixed, but the emulsion in which the degree of internal chemical sensitization has been increased can have no sufficient efficiency for the formation of positive im-

ages, can also have no sufficient maximum density despite a mixed emulsion, and has been desired to achieve a still higher maximum density.

Japanese Patent Publications Open to Public Inspection (hereinafter referred to as Japanese Patent O.P.I. Publications) Nos. 111938/1983 and 77436/1984 discloses the mixing and double layer coating of a core-shell emulsion and a fine grain emulsion. The fine grain emulsion, however, can not form an image when used alone, and is used merely to improve covering power, so that it can not enhance the photographic performances possessed by respective emulsions, also resulting in a higher minimum density.

Also, in the direct-positive silver halide photographic light-sensitive materials, developing is carried out in the presence of a fogging agent after imagewise exposure, thereby forming a fog nucleus in silver halide emulsion and carrying out the development, so that their photographic performances greatly depend on the conditions under which the emulsion is fogged, i.e., the type and amount of fogging agents or the character of developing solutions. Accordingly, in regard to, for example, the developing solutions, there is a demand for a direct-positive silver halide photographic light-sensitive material that has stable photographic performances against changes in composition or the lowering of developing ability owing to running or fatigue.

Moreover, in the direct-positive silver halide photographic light-sensitive materials, an attempt to reproduce with fidelity the lightness of objects results in requirement of a soft gradation performance having a broad exposure latitude. Hence, for example, the broad exposure latitude is obtained, or further the gradation is controlled, by mixing internal latent image silver halide grains having different grain size and substantially the same light-sensitive wavelength or by overlapping them by coating in different layers. In this occasion, however, because of employment of the grains having different grain size, the development proceeds in a different manner for each grain having different grain size, and for this reason the development proceeds slowly in respect of larger grains and the development proceeds quickly in respect of smaller grains, thus sometimes resulting in the so-called poorly continuous gradation that the gradation greatly differs at the toe and the shoulder of the characteristic curve thereof, particularly in the direct-positive color photographic light-sensitive materials, this point has not been sufficiently settled despite the importance of the balance in the toe portion of the characteristic curve. Satisfactory results are not necessarily obtained also in regard to the stability of direct-positive silver halide photographic light-sensitive materials, when the development conditions have been varied.

As a measure relating to this stability against the variation of developing conditions, some methods have been proposed in which emulsion grains are made development-active, e.g., the emulsion grains are made to have a small grain size, or a coupler capable of rapidly reacting with an oxidized developing agent to used, but these are still not only insufficient for obtaining always stable performances, but also accompanied with an increase in minimum density, undesirably.

**SUMMARY OF THE INVENTION**

An object of the present invention is to provide a direct-positive silver halide photographic light-sensitive material that have a good image quality having a suffi-

ciently high maximum density, yet having a sufficiently low minimum density, and at the same time not only have a broad exposure latitude, i.e., have a broad gradient and good gradation reproducibility, but also have the photographic performance that affords a stable balance of the gradation at the toe of the characteristic curve against variations of developing conditions, and a method of processing the same.

The above object of the present invention was achieved by a direct-positive silver halide photographic light-sensitive material which comprises a support having thereon a blue-sensitive emulsion layer, a green-sensitive emulsion layer and a red-sensitive emulsion layer, and is capable of obtaining a positive image by developing with a color developer in the presence of a fogging agent after exposure to light;

wherein the green-sensitive emulsion layer comprises;

silver halide grains having at least two peaks on the grain size distribution curve thereof, where the grain size corresponding to the smallest grain size peak among said at least two peaks is not more than 0.3  $\mu\text{m}$ ; and

at least one of the magenta couplers represented by Formula (M-I).



Formula (M-I)

wherein Z represents a group of non-metal atoms necessary to complete a nitrogen-containing heterocyclic ring which may have a substituent; X represents a hydrogen atom or a group capable of being split off upon reaction with the oxidized product of a color developing agent; and R represents a hydrogen atom or a substituent.

The above object was also achieved by a method of processing a direct-positive silver halide photographic light-sensitive material, comprising subjecting the above light-sensitive material to color development in the presence of a fogging agent.

#### DETAILED DESCRIPTION OF THE INVENTION

The direct-positive silver halide photographic light-sensitive material (hereinafter "direct-positive light-sensitive material") according to the present invention has at least one blue-sensitive emulsion layer, green-sensitive emulsion layer and red-sensitive emulsion layer, respectively, on a support. In the present light-sensitive material, each layer of at least one blue-sensitive emulsion layer, green-sensitive emulsion layer and red-sensitive emulsion layer, respectively, may comprise a single layer or plural layers. In the case of plural layers, a non-light-sensitive emulsion layer or other light-sensitive emulsion layer may be provided between the layer nearest to the support and the layer farthest from the support. The above green-sensitive emulsion layer comprises grains having at least two peaks in the grain size distribution curve of the silver halide grains contained in said layer. In the case when the green-sensitive emulsion layer comprises plural layers, the grains refer to those having at least two peaks in the grain size distribution curve obtained by measuring the grain size distribution curve of the whole silver halide grains of the re-

spective silver halide grains contained in the plural layers coated per unit area.

In the following, the manner by which the grain size distribution is measured will be described in detail. In the case of spherical silver halide grains, the grain size of the silver halide emulsion grains mentioned here refers to the diameter of a grain. In the case of silver halide grains having forms other than the spherical form, it means the diameter obtained when the projected image of a grain has been calculated into a round image having the same area. The grain size can be obtained, for example, by taking a photograph with enlargement of from 10,000 to 50,000 magnifications using an electron microscope and actually measuring the diameter of the grains on the resulting print or the area obtained by the projected image. (The grains to be measured are selected at random in the number of not less than 1,000.)

The position at which  $n_i \times r_i^3$  shows a maximum value when the product of frequency  $n_i$  of a grain having grain size  $r_i$ , and  $r_i^3$ , i.e.,  $n_i \times r_i^3$ , is plotted with respect to  $r_i$  is defined to be the peak in the grain size distribution curve in the present invention.

The silver halide grains contained in the green-sensitive emulsion layer according to the present invention are required to have at least two peaks in the grain size distribution curve of the grains, but may more preferably have at least three peaks in the grain size distribution curve.

In the present invention, there are no particular limitations on the size of the respective peaks in the above peaks of the grain size distribution curve, but the weight of silver halide grains included in a grain size range of  $\pm 20\%$  centering on the grain size at the respective peaks may preferably comprise not less than 5%, more preferably not less than 10%, of the weight of the whole silver halide grains.

In the grain size distribution curve of the silver halide grains in the present invention, there are no particular limitations on the extent to which any adjacent peaks stand apart in their grain size, but at least the grain size at the peaks stands not less than 10% apart from the grain size based on a greater grain size.

The green-sensitive emulsion layer may preferably contain at least two kinds of silver halide emulsions having different average grain size. In the case when the green-sensitive emulsion layer comprises a single layer, the layer contains, in a preferred embodiment, at least two kinds of silver halide emulsions having different average grain size. Also, in the case when the green-sensitive emulsion layer comprises plural layers, each layer may have the same or different grain size distribution, so long as the grains have at least two peaks in the grain size distribution curve as a whole.

In a preferred embodiment of the present invention, at least two kinds of silver halide emulsion different in average grain size are separately contained in different green-sensitive emulsion layers.

For instance, in a case that the green-sensitive emulsion layer is comprises two emulsion layers and one of which contains an emulsion comprising silver halide grains having a smaller average grain size and the other of which contains silver halide grains having a larger average grain size, the size distribution curve of the above whole grains including the grains of a smaller average grain size and the grains of a larger average grain size coated in an unit area has at least two peaks.

Among at least two peaks in the grain size distribution curve of the silver halide grains contained in the green-sensitive emulsion layer according to the present invention, the grain size corresponding to the smallest grain size peak is not more than 0.3  $\mu\text{m}$ , preferably 0.05  $\mu\text{m}$  to 0.3  $\mu\text{m}$ , and, among the above at least two peaks, there are no particular limitations on the grains size at the peaks other than the smallest grain size peak, but the grain size may preferably be not more than 1.5  $\mu\text{m}$ . More preferably it may be not more than 1.0  $\mu\text{m}$ , and particularly preferably not more than 0.7  $\mu\text{m}$ .

The silver halide emulsion contained in the green-sensitive emulsion layer according to the present invention contain a magenta coupler represented by Formula (M-I).



Formula (M-I)

In the magenta coupler represented by the above Formula (M-I), Z represents a group of non-metal atoms necessary to complete a nitrogen-containing heterocyclic ring, and the ring formed by said Z may have a substituent.

X represents a hydrogen atom or a group capable of being split off upon reaction with the oxidized product of a color developing agent.

R represents a hydrogen atom or a substituent.

There are no particular limitations on the substituent represented by R, but it typically includes groups such as alkyl, aryl, anilino, acylamino, sulfonamide, alkylthio, arylthio, alkenyl and cycloalkyl. Besides these, it also includes a halogen atom, groups such as cycloalkenyl, alkynyl, a heterocyclic ring, sulfonyl, sulfinyl, phosphonyl, acyl, carbamoyl, sulfamoyl, cyano, alkoxy, aryloxy, heterocyclic oxy, siloxy, acyloxy, carbamoyloxy, amino, alkylamino, imido, ureido, sulfamoylamino, alkoxycarbonylamino, aryloxycarbonylamino, alkoxycarbonyl, aryloxycarbonyl and heterocyclic thio, a spiro compound residual group, and a bridged hydrocarbon compound residual group.

The above alkyl group represented by R may preferably include those having 1 to 32 carbon atoms, which may be either straight-chain or branched.

The aryl group represented by R may preferably include a phenyl group.

The acylamino group represented by R includes an alkylcarbonylamino group and an arylcarbonylamino group.

The sulfonamide group represented by R includes an alkylsulfonylamino group and an arylsulfonylamino group.

The alkyl component or aryl component in the alkylthio group or arylthio group represented by R includes the above alkyl group or aryl group represented by R.

The alkenyl group represented by R may preferably include those having 2 to 32 carbon atoms; and the cycloalkyl group, those having 3 to 12 carbon atoms, and particularly 5 to 7 carbon atoms. The alkenyl group may be either straight-chain or branched.

The cycloalkenyl group represented by R may preferably include those having 3 to 12 carbon atoms, and particularly preferably 5 to 7 carbon atoms.

The sulfonyl group represented by R includes an alkylsulfonyl group and an arylsulfonyl group;

the sulfinyl group includes an alkylsulfinyl group and an arylsulfinyl group;

the phosphonyl group includes an alkylphosphonyl group, an alkoxyphosphonyl group, an aryloxyphosphonyl group and an arylphosphonyl group;

the acyl group includes an alkylcarbonyl group and an arylcarbonyl group;

the carbamoyl group includes an alkylcarbamoyl group and an arylcarbamoyl group;

the sulfamoyl group includes an alkylsulfamoyl group and an arylsulfamoyl group;

the acyloxy group includes an alkylcarbonyloxy group and arylcarbonyloxy group;

the carbamoyloxy group includes an alkylcarbamoyloxy group and an arylcarbamoyloxy group;

the ureido group includes an alkylureido group and an arylureido group;

the sulfamoylamino group includes an alkylsulfamoylamino group and an arylsulfamoylamino group;

the heterocyclic ring may preferably include those of 5 to 7 members, specifically including a 2-furyl group, a 2-thienyl group, 2-pyrimidinyl group and 2-benzothiazolyl group;

the heterocyclic oxy group may preferably include those having a heterocyclic ring of 5 to 7 members, including, for example, a 3,4,5,6-tetrahydropyran-2-oxy group and a 1-phenyltetrazole-5-oxy group;

the heterocyclic thio group may preferably include a heterocyclic thio group of 5 to 7 members, including, for example, a 2-pyridylthio group, a 2-benzothiazolylthio group and a 2,4-diphenoxyl-1,3,5-triazole-6-thio group;

the siloxy group includes a trimethylsiloxy group, a triethylsiloxy group and a dimethylbutylsiloxy group;

the imido group includes a succinimido group, a 3-heptadecylsuccinimido group, a phthalimido group and a glutalimido group;

the spiro compound residual group includes spiro[3.3]heptan-1-yl; and

the bridged hydrocarbon compound residual group includes bicyclo[2.2.1]heptan-1-yl, tricyclo[3.3.1.1<sup>3,7</sup>]dec-1-yl and 7,7-dimethylbicyclo[2.2.1]heptan-1-yl.

The group represented by X, capable of being split off through the reaction with an oxidized product of a color developing agent, may include, for example, a halogen atom such as a chlorine atom, a bromine atom or a fluorine atom, and groups such as alkoxy, aryloxy, heterocyclic oxy, acyloxy, sulfonyloxy, alkoxy carbonyloxy, aryloxycarbonyl, alkyloxaloyloxy, alkoxyoxaloyloxy, alkylthio, arylthio, heterocyclo thio, alkyloxythiocarbonylthio, acylamino, sulfonamido, a nitrogen-containing heterocyclic ring bonded with a N atom, alkyloxycarbonylamino, aryloxycarbonylamino, carboxyl, and



(R1' represents the same as defined for the above R, and Z', the same as defined for the above Z; and R2' and R3' each represent a hydrogen atom, an aryl group, an alkyl group or a heterocyclic group.), but preferably includes a halogen atom, particularly a chlorine atom.

The nitrogen-containing heterocyclic group formed by Z or Z' may include a pyrazole ring, an imidazole ring, a triazole ring or a tetrazole ring, and the substituent on the above ring may have may include those described for the above R.

The coupler represented by Formula (M-I) is more specifically represented, for example, by the following Formulas (M-II) to (M-VII).



Formula (M-II)



Formula (M-III)



Formula (M-IV)



Formula (M-V)



Formula (M-VI)



Formula (M-VII)

In the above Formulas (M-II) to (M-VII), R<sub>1</sub> to R<sub>8</sub> and X represent the same as defined for the above R and X.

Among Formula (M-I), preferred is the one represented by Formula (M-VIII) shown below.



Formula (M-VIII)

wherein R<sub>1</sub>, X and Z<sub>1</sub> represent the same as defined for R, X and Z in Formula (M-I).

Among the magenta couplers represented by the above Formulas (M-II) to (M-VII), a preferred magenta coupler is the magenta coupler represented by Formula (M-II) or (M-III) and particularly preferred is one represented by Formula (II).

Most preferred as the substituent R or R<sub>1</sub> on the above heterocyclic ring is a substituent represented by Formula (M-IX) shown below.



wherein R<sub>9</sub>, R<sub>10</sub> and R<sub>11</sub> each represent the same as defined for the above R.

Any two of the above R<sub>9</sub>, R<sub>10</sub> and R<sub>11</sub>, for example, R<sub>9</sub> and R<sub>10</sub>, may also combine to form a saturated or unsaturated ring as exemplified by cycloalkane, cycloalkene and a heterocyclic ring, and R<sub>11</sub> may further be combined to said ring to constitute a bridged hydrocarbon compound residual group.

Particularly preferred in Formula (M-IX) are;

(i) the case when at least two of R<sub>9</sub> to R<sub>11</sub> are alkyl groups; and

(ii) the case when one of R<sub>9</sub> to R<sub>11</sub>, for example, R<sub>11</sub>, is a hydrogen atom, and other two, R<sub>9</sub> and R<sub>10</sub>, are combined to form cycloalkyl together with the route carbon atom.

Further particularly preferred in (i) is the case when any two of R<sub>9</sub> to R<sub>11</sub> are alkyl groups and the remaining one is a hydrogen atom or an alkyl group.

Also, the substituent the ring formed by Z in Formula (M-I) or the ring formed by Z<sub>1</sub> in Formula (M-VIII) may have, and R<sub>2</sub> to R<sub>8</sub> in Formulas (M-II) to (M-VI) may preferably include those represented by Formula (M-X) shown below.



Formula (M-X)

In the formula, R<sup>1</sup> represents an alkylene group, and R<sup>2</sup> represents an alkyl group, a cycloalkyl group or an aryl group.

The alkylene group represented by R<sup>1</sup> may preferably have two or more, more preferably 3 to 6, carbon atoms at the straight-chain moiety, regardless of being straight-chain or branched.

The cycloalkyl group represented by R<sup>2</sup> may preferably include those of 5 or 6 members.

Typical examples of the compounds according to the present invention are shown below.



-continued



3



4



5



6



7



8



9

4,943,518

11

12

**-continued**

10



11



12



13



14



15



16



17



-continued



-continued

27



28



29



30



31



32



33



34



-continued

35



36



37



38



39



40



41



4,943,518

19

20

-continued



-continued

50



51



52



53



54



55



56



57



58



-continued



x:y = 50:50

59



x:y = 50:50

60

In addition to the above typical examples of the compounds according to the present invention, examples of the compounds according to the present invention may also include the compounds shown as Nos. 1 to 4, 6, 8 to 17, 19 to 24, 26 to 43, 45 to 59, 61 to 104, 10 to 121, 123 to 162 and 164 to 223 among the compounds described at pages 66 to 122 of the specification of Japanese Patent O.P.I. Publication No. 166339/1987.

The above couplers can be synthesized by making reference to Journal of the Chemical Society, Perkin I (1977), 2047-2052, U.S. Pat. No. 3,725,067, Japanese Patent O.P.I. Publications Nos. 99437/1984, 42045/1983, 162548/1984, 171956/1984, 33552/1985, 43659/1985, 172982/1985 and 190779/1985, etc.

The magenta couplers of the present invention can be used usually in the range of from  $1 \times 10^{-3}$  mol to 1 mol, and preferably from  $1 \times 10^{-2}$  mol to  $8 \times 10^{-1}$  mol, per mol of silver halide.

The couplers of the present invention can also be used in combination with magenta couplers of different types.

In green-sensitive layer of the photographic material of the present invention, at least two silver halide emulsions different in average grain size are separately coated in plural layers, or at least one emulsion having at least two peaks in its grain size distribution curve is coated in one or more layers.

Methods of preparing the silver halide emulsion used in the present invention will be described below in detail.

One of the methods of preparing emulsions so as to give a desired grain size distribution is a method in which at least two kinds of emulsions having different grain size are mixed. In this instance, the respective emulsions may preferably comprise a monodisperse emulsion.

In another method of preparing an emulsion, the emulsion is so prepared that the grain size distribution curve of the present invention can be obtained by using a single emulsion, where, for example, silver ions and halide ions are fed to a seed emulsion, and an additional seed emulsion is added when silver halide crystals have grown to have a given particle size in a monodisperse state, and thereafter silver ions and halide ions are again fed, so that the silver halide grains having two peaks in

25

30

35

40

45

50

55

60

65

the grain size distribution curve in the present invention can be obtained.

In still another method, silver halide grains are made to grow under such a condition or rate of addition that any new silver halide nucleus may not be formed, thereafter silver halide nuclei are made to grow under such a condition or rate of addition that maV temporarily cause the formation of new nuclei of silver halide grains and thereafter the rate of addition is so controlled as not to again form any new silver halide nucleus, so that the silver halide grains having two peaks can also be prepared.

The silver halide grains used in the present invention may be those obtained by any of an acidic method, a neutral method and an ammoniacal method. The grains may be grown at one time, or may be grown after making seed grains. The method of making seed grains and the method of growing them maV be the same or different. The silver halide emulsion containing such silver halide grains may be prepared either by simultaneously mixing halide ions and silver ions or by mixing any one of them into an aqueous solution in which the other of them is present. The grains may also be made to grow by simultaneously adding halide ions and silver ions while controlling the pH and pAg in a mixing vessel, taking into consideration the critical growth rate of silver halide crystals. This method can yield silver halide grains having regular crystal forms and nearly uniform grain size. It is also possible to change the halogen composition of the grains with use of a conversion process after the growth.

The silver halide grain according to the present invention may comprise at least two phases, more specifically, at least two phases having different halogen composition from each other, and one of the phases positioned at the outermost side maV only cover at least part of the other phase. The grain may have the so-called core/shell structure, in which a second phase forms a core and a first phase serves as a shell to cover the core, or have the structure in which the first phase covers part of the second phase.

The silver halide grain according to the present invention may be constituted of three or more layers. For example, it may be a silver halide grains having a three layer constitution comprising a core serving as the innermost central nucleus, an internal shell that covers the

core, and the outermost shell layer that covers the internal shell. Hereinafter, to simplify the description, the grain having the two layer structure will be taken up to make description regarding a first phase positioned at the outermost side as the shell layer, and a second phase adjacent thereto as the core. However, the silver halide grain of the present invention may not be limited to the grain of two-layer structure.

The core of the silver halide grain according to the present invention may preferably contain less silver chloride than the silver chloride contained in the shell layer.

The core may preferably be mainly comprised of silver bromide, and may further contain silver chloride and/or silver iodobromide. The silver halide grain that forms the core may be of any form, as exemplified by a cube, a regular octahedron, a dodecahedron or a tetradecahedron, these of which may be used in a mixed state, and also may be a spherical, plate-like or formless grain, these of which may be used in an appropriately mixed state. In working the present invention, the average grain size and grain size distribution of the silver halide grains that constitute the core or internal shell can be made to vary in a vast range depending on the desired photographic performances, but the grain size distribution with a narrower distribution is more preferred. Specifically, 90% by weight of the silver halide grains that constitute the core may preferably have a grain size included in the range of plus or minus 40%, and more preferably plus or minus 30%, of the average grain size.

In other words, the silver halide grains that constitute the cores may preferably be substantially monodisperse.

The silver halide grains whose cores are monodisperse are herein meant to be those in which, in the silver halide grains that constitute the cores, the weight of silver halide grains included in a grain size range of  $\pm 20\%$  centering on an average grain size  $r$  comprise not less than 60%, preferably not less than 70%, and particularly preferably not less than 80%, of the weight of the whole silver halide grains.

Here, the average grain size  $r$  means such a grain size  $r$  that the product of frequency  $n_i$  of a grain having grain size  $r_i$ , and  $r_i^3$ , i.e.,  $n_i \times r_i^3$ , may come to be maximum (effective number: three figures; minimum figures are rounded off).

The grain size mentioned here also refers to the diameter of a grain in the case of spherical silver halide grains. In the case of silver halide grains having forms other than the spherical form, it refers to the diameter obtained when the projected image of a grain has been calculated into a round image having the same area.

As methods of preparing the above monodisperse core emulsions, the double-jet method can be used which is disclosed, for example, in Japanese Patent Examined Publication No. 36890/1973, and Japanese Patent O.P.I. publications No. 48520/1979 and No. 65521/1979. Besides this, the premix method can be also used which is described in Japanese Patent O.P.I. Publication No. 158220/1979.

The core may preferably have less lattice defects, which is disclosed, for example, in U.S. Pat. No. 2,592,250. The emulsion prepared by a conversion method is not suitable as the core. The grains prepared by the above double jet method while controlling the pH and pAg during preparation have less lattice defects, and are preferred as the core.

The core can be prepared in the presence of a silver halide solvent. There can be used thioethers disclosed in U.S. Pat. No. 3,574,628 thiourea derivatives disclosed in Japanese Patent O.P.I. Publication No. 77737/1980, and imidazoles disclosed in Japanese Patent O.P.I. Publication No. 100717/1979. In a preferred embodiment of the present invention, it is also preferred to use ammonia as the silver halide solvent.

In the silver halide grains according to the present invention, the shell layer may preferably cover not less than 50% of the surface area of the grain that constitutes the core. The shell layer may contain silver bromide or silver iodide so far as any photographic performances are adversely affected. Part of the shell layer may be converted into silver bromide or silver iodide by using a little amount of a water-soluble bromide or iodide.

The shell layer may entirely cover the core, or may selectively cover part of the core, but may preferably cover not less than 50% of the surface area of the core. More preferably, it may entirely cover the core.

As methods of forming the shell layer, the above double jet method or premix method can be used. It can also be formed by mixing finely particulate silver halide into an emulsion containing the grain that constitutes the core, followed by Ostwald ripening.

In working the present invention, the cores of silver halide grains may be chemically sensitized, or doped with metal ions, or applied with both of them, or applied with none of the both at all.

Employable as the chemical sensitization are sulfur sensitization, gold sensitization, reduction sensitization, noble metal sensitization, and sensitizing methods comprising any combination of these sensitizing methods. Usable as sulfur sensitizers are thiosulfate, thioureas, thiazoles, rhodanines, and other compounds. Such methods are described, for example, in U.S. Pat. Nos. 1,574,944, 1,623,499, 2,410,689 and U.S. Pat. No. 3,656,955.

The cores of the silver halide grains used in working the present invention can be sensitized with a water-soluble gold compound or can be sensitized with use of a reducing sensitizer, as described, for example, in U.S. Pat. Nos. 2,399,083, 2,597,856 and U.S. Pat. No. 2,642,361. As to such methods, reference can be made, for example, on the descriptions in U.S. Pat. Nos. 2,487,850, 2,518,698 and U.S. Pat. No. 2,983,610.

It is further possible to carry out noble metal sensitization with use of noble metal compounds as exemplified by platinum, iridium and palladium. As to such methods, reference can be made, for example, on the descriptions in U.S. Pat. No. 2,448,060 and British Pat. No. 618,061.

The cores of the silver halide grains can also be doped with metal ions. To dope the cores with metal ions, metal ions can be added, for example, as water-soluble salts of metal ions in any course during which the grains for cores are formed. Preferred examples of the metal ions include metal ions such as iridium, lead, antimony, bismuth, gold, osmium and rhodium. These metal ions may preferably be used in a concentration of  $1 \times 10^{-3}$  to  $1 \times 10^{-4}$  mol per mol of silver.

Provided that those used as the cores of silver halide grains may not be subjected to the above chemical sensitization treatments or doping with metal ions. In such instances, sensitivity centers are presumed to be produced by, e.g., forming crystal distortion at the interface between the core and shell layer in the course of

covering the grains of cores with the shell layers. In relation thereto, reference can be made on the descriptions in U.S. Pat. Nos. 3,935,014 and 3,957,488.

The silver halide emulsion used in the present invention can be chemically sensitized by commonly available methods at any stages during preparation. The silver halide grains of the present invention can further occlude polyvalent metal ions in the insides of grains. preferred examples of the polyvalent metal ions include metal ions such as iridium, lead, antimony, bismuth, gold, platinum, osmium and rhodium. 10

The silver halide grains according to the present invention may preferably be not chemically sensitized on the grains surfaces, or, if sensitized, sensitized to a slight degree. 15

In the direct-positive silver halide photographic light-sensitive material of the present invention, internal latent image silver halide grains not previously fogged on the surfaces can be used. Here, what is meant bV the internal latent image silver halide grains not previously fogged on the surfaces is that the density obtained when test pieces comprising transparent film supports coated with the above emulsion to a thickness of mgAg/cm<sup>2</sup> were developed at 20° C. for 10 minutes without exposure to light, using the following surface developing solution A, is not more than 0.6, and preferably not more than 0.4. 20

|                                      |       |    |
|--------------------------------------|-------|----|
| Metol                                | 2.5 g | 30 |
| l-Ascorbic acid                      | 10 g  |    |
| NaBO <sub>2</sub> .4H <sub>2</sub> O | 35 g  |    |
| KBr                                  | 1 g   |    |
| Made up by adding water, to          | 1 l   |    |

The emulsion containing the silver halide grains according to the present invention can give a sufficient density when a test piece prepared in the following manner was exposed to light and thereafter developed with an internal developing solution B having the following recipe. 35 40

|                                |        |    |
|--------------------------------|--------|----|
| Metol                          | 2 g    | 45 |
| Sodium sulfite (anhydrous)     | 90 g   |    |
| Hydroquinone                   | 8 g    |    |
| Sodium carbonate (monohydrate) | 52.5 g |    |
| KBr                            | 5 g    |    |
| KI                             | 0.5 g  |    |
| Made up by adding water, to    | 1 l    |    |

To describe in a further specific way, when a part of the above test pieces is exposed to light to a light intensity scale over a given time not exceeding about 1 second and developed at 20° C. for 10 minutes using the internal developing solution B, shown is a maximum density at least 5 times, and preferably at least 10 times, 50 55 greater than the density obtained when another part of the test pieces, exposed to light under the same conditions, was developed at 20° C. for 10 minutes using the surface developing solution A.

In the processing method of the present invention, 60 the light-sensitive material is developed in the presence of a fogging agent.

The developing solutions used here may preferably contain a phosphoric acid compound.

Any compounds can be used as the phosphoric acid 65 compound, typically including phosphoric acid, orthophosphoric acid, all sorts of polyphosphoric acids, and derivatives such as salts of these. More specifically,

usable phosphoric acid compounds include those represented by the following Formula (P-I), (P-II) or (P-III).



wherein, A<sup>1</sup> to A<sup>7</sup> each represent a hydrogen atom, an alkali metal atom or an alkyl group; and m and n each represent an integer of 1 to 20.

Of the phosphoric acid compounds represented by Formula (P-I), (P-II) or (P-III), preferably used in the present invention are the compounds represented by any of the following Formulas (P-IV) to (P-XI).



wherein M represents a hydrogen atom or an alkali metal atom; and m and n each represent an integer of 1 to 20. 20



wherein E represents a substituted or unsubstituted alkylene group, a cycloalkylene group, a phenylene group, —R<sub>27</sub>—, —OR<sub>27</sub>—, —R<sub>27</sub>—OR<sub>27</sub>—, —R<sub>27</sub>—OR<sub>27</sub>— or R<sub>27</sub>ZR<sub>27</sub>—; Z represents >N—R<sub>27</sub>—B<sub>6</sub> or >N—B<sub>6</sub>; R<sub>21</sub> to R<sub>27</sub> each represent a substituted or unsubstituted alkylene group; B<sub>1</sub> to B<sub>6</sub> each represent a hydrogen atom, —OH, —COOM, —PO<sub>3</sub>M<sub>2</sub>, where at least one of B<sub>1</sub> and B<sub>6</sub> represents —PO<sub>3</sub>M<sub>2</sub>, at least one of B<sub>2</sub> to B<sub>5</sub> represents —PO<sub>3</sub>M<sub>2</sub>; and M represents a hydrogen atom or an alkali metal atom.



wherein R<sub>28</sub> represents a lower alkyl group, an aryl group, an aralkyl group, a nitrogen-containing 6-membered ring group (having —OH, —OP or —COOM as a substituent); and M represents a hydrogen atom or an alkali metal atom.



wherein R<sub>29</sub> to R<sub>31</sub> each represent a hydrogen atom, —OH, a lower alkyl group which is unsubstituted, or having —OH, —COOM or —PO<sub>3</sub>M<sub>2</sub> as a substituent; C<sub>1</sub> to C<sub>3</sub> each represent a hydrogen atom, —OH, —COOM, —PO<sub>3</sub>M<sub>2</sub> or —Nj<sub>2</sub>, where j represents a hydrogen atom, a lower alkyl group, C<sub>2</sub>H<sub>5</sub>OH or —PO<sub>3</sub>M<sub>2</sub>; M represents a hydrogen atom or an alkali metal atom; and n and m each represent 0 or 1.





-continued



(P-31)

5



(P-32) 10

15



(P-33)

20



(P-34)

25



(P-35)

30



(P-36)

35



(P-37)

40



(P-38)

45



(P-39)

50



(P-40)

55



(P-51)

60

65

65

(P-41)

(P-42)

(P-43)

(P-44)

(P-45)

(P-46)

(P-47)

(P-48)

(P-49)

(P-50)

(P-51)

(P-52)

-continued



The above phosphoric acid compounds may preferably be used in an amount of from 3 g to 200 g, and more preferably from 5 g to 10 g, per liter of the developing solution. In the present invention, it is preferred to use a developing solution with the pH of 9.5 to 12.0.

In the processing method used in the present invention, the color developing solution may preferably contain substantially no hydroxylamine except derivatives thereof.

Incorporation of a hydroxylamine derivative represented by the following Formula (HA) into the developing solution used in the present invention can bring about not only a better exhibition of the effect aimed in the present invention but also a low suppressed fog density at unexposed portions of light-sensitive materials. Accordingly, this may preferably be used in combination in the present invention.



Formula (HA)

In the formula R<sub>41</sub> and R<sub>42</sub> each represent an alkyl group or a hydrogen atom. Provided that both R<sub>41</sub> and R<sub>42</sub> are not hydrogen atoms at the same time. R<sub>41</sub> and R<sub>42</sub> may also combine to form a ring.

In (HA), R<sub>41</sub> and R<sub>42</sub> each represent an alkyl group or a hydrogen atom, which are not hydrogen atoms at the same time, but the alkyl groups represented by R<sub>41</sub> and R<sub>42</sub> may be the same or different, and may preferably each represent an alkyl group having 1 to 3 carbon atoms. The alkyl groups represented by R<sub>41</sub> and R<sub>42</sub> includes those having a substituent, and R<sub>41</sub> and R<sub>42</sub> may combine to constitute a ring. for example, may constitute a heterocyclic ring such as pipéridine or morphine.

Specific compounds of the hydroxylamine derivative represented by Formula (HA) are described in U.S. Pat. Nos. 3,287,125, 3,293,034, U.S. Pat. No. 3,287,124 and so forth, but particularly preferred exemplary compounds are shown below.

Exemplary Compound No.

|      | R <sub>41</sub>                    | R <sub>42</sub>                    |
|------|------------------------------------|------------------------------------|
| A-1  | -C <sub>2</sub> H <sub>5</sub>     | -C <sub>2</sub> H <sub>5</sub>     |
| A-2  | -CH <sub>3</sub>                   | -CH <sub>3</sub>                   |
| A-3  | -C <sub>3</sub> H <sub>7</sub> (n) | -C <sub>3</sub> H <sub>7</sub> (n) |
| A-4  | -C <sub>3</sub> H <sub>7</sub> (i) | -C <sub>3</sub> H <sub>7</sub> (i) |
| A-5  | -CH <sub>3</sub>                   | -C <sub>2</sub> H <sub>5</sub>     |
| A-6  | -C <sub>2</sub> H <sub>5</sub>     | -C <sub>3</sub> H <sub>7</sub> (i) |
| A-7  | -CH <sub>3</sub>                   | -C <sub>3</sub> H <sub>7</sub> (i) |
| A-8  | -H                                 | -C <sub>2</sub> H <sub>5</sub>     |
| A-9  | -H                                 | -C <sub>3</sub> H <sub>7</sub> (n) |
| A-10 | -H                                 | -CH <sub>3</sub>                   |

(P-53)

-continued



5

Exemplary Compound No.

|    |      |                                                  |                                                               |
|----|------|--------------------------------------------------|---------------------------------------------------------------|
| 10 | A-11 | -H                                               | -C <sub>3</sub> H <sub>7</sub> (i)                            |
|    | A-12 | -C <sub>2</sub> H <sub>5</sub>                   | -C <sub>2</sub> H <sub>4</sub> OCH <sub>3</sub>               |
|    | A-13 | -C <sub>2</sub> H <sub>4</sub> OH                | -C <sub>2</sub> H <sub>4</sub> OH                             |
|    | A-14 | -C <sub>2</sub> H <sub>4</sub> SO <sub>3</sub> H | -C <sub>2</sub> H <sub>5</sub>                                |
| 15 | A-15 | -C <sub>2</sub> H <sub>4</sub> COOH              | -C <sub>2</sub> H <sub>4</sub> COOH                           |
|    | A-16 |                                                  |                                                               |
|    | A-17 |                                                  |                                                               |
| 20 | A-18 |                                                  |                                                               |
| 25 | A-19 |                                                  |                                                               |
| 30 | A-20 | R <sub>41</sub>                                  | R <sub>42</sub>                                               |
|    | A-21 | -CH <sub>3</sub>                                 | -C <sub>2</sub> H <sub>4</sub> OCH <sub>3</sub>               |
|    | A-22 | -C <sub>2</sub> H <sub>4</sub> OCH <sub>3</sub>  | -C <sub>2</sub> H <sub>4</sub> OC <sub>2</sub> H <sub>5</sub> |
|    | A-23 | -C <sub>3</sub> H <sub>6</sub> OCH <sub>3</sub>  | -C <sub>3</sub> H <sub>6</sub> OCH <sub>3</sub>               |
|    | A-24 | -C <sub>2</sub> H <sub>5</sub>                   | -C <sub>2</sub> H <sub>4</sub> OC <sub>2</sub> H <sub>5</sub> |
|    | A-25 | -C <sub>3</sub> H <sub>7</sub>                   | -C <sub>2</sub> H <sub>4</sub> OCH <sub>3</sub>               |
|    | A-26 | -CH <sub>3</sub>                                 | -C <sub>2</sub> H <sub>4</sub> OC <sub>2</sub> H <sub>5</sub> |
|    | A-27 | -CH <sub>3</sub>                                 | -CH <sub>2</sub> OCH <sub>3</sub>                             |
|    | A-28 | -C <sub>2</sub> H <sub>5</sub>                   | -CH <sub>2</sub> OC <sub>2</sub> H <sub>5</sub>               |
|    | A-29 | -CH <sub>2</sub> OCH <sub>3</sub>                | -CH <sub>2</sub> OCH <sub>3</sub>                             |
| 35 | A-30 | -C <sub>2</sub> H <sub>5</sub>                   | -C <sub>2</sub> H <sub>4</sub> OC <sub>2</sub> H <sub>7</sub> |
|    | A-31 | -C <sub>3</sub> H <sub>6</sub> OCH <sub>3</sub>  | -C <sub>3</sub> H <sub>6</sub> OC <sub>2</sub> H <sub>7</sub> |

50 These compounds are usually used in the form of hydrochloride, sulfate, p-toluenesulfonate, oxalate, phosphate or acetate, or in the free form.

55 The compound represented by Formula (HA) of the present invention is contained in the color developing solution in a concentration of usually from 0.2 g/l to 50 g/l, preferably from 0.5 g/l to 30 g/l, and more preferably from 1 g/l to 15 g/l.

60 The compound represented by Formula (HA) may also be used alone or in combination of two or more types.

65 The direct-positive silver halide photographic light-sensitive material of the present invention may preferably contain a compound represented by the following Formula (HQ) in any layer of hydrophilic colloid layers.

This Formula (HQ) is as shown below.



In Formula (HQ), R<sub>51</sub> and R<sub>52</sub> each represent a hydrogen atom or an alkyl group, and each alkyl group of R<sub>51</sub> and R<sub>52</sub> has the carbon atom number of not more than 5.

Specifically, the compounds shown in the following (A) to (H) are preferred as the compound represented by Formula (HQ). Provided that those which can be used in the present invention are by no means particularly limited to these compounds

(Examples of compounds)



(A)

20 The amount of this compound to be added in at least any one layer of the photographic component layers may preferably range from 0.001 to 0.50 g/m<sup>2</sup>, and more preferably from 0.005 to 0.20 g/m<sup>2</sup>. Also, the above compounds may be used alone or may be mixed by arbitrarily selecting two or more compounds. It is also possible to use a quinone derivative having not less than 5 carbon atoms by adding it to the compound represented by the above Formula (HA), so long as the effect of the present invention may not be impaired. In either case of these, the amount of the compound to be used even as a mixture may preferably range from 0.001 to 0.50 g/m<sup>2</sup>.

(B) 25 The silver halide emulsion can be optically sensitized using sensitizing dyes commonly used. Combination of sensitizing dyes used in supersensitization of internal latent image silver halide emulsions, negative silver halide emulsions, etc. is also useful for the silver halide emulsion of the present invention. As to the sensitizing dyes, reference can be made on Research Disclosures No., 15162 and No. 17643.

(C) 30 In instances in which direct-positive images are obtained by using the direct-positive silver halide photographic light-sensitive material of the present invention, the direct positive images can be readily obtained by carrying out imagewise exposure (the so-called photography, i.e., exposing a light-sensitive material to light to form an image) according to a usual method, followed by surface development. More specifically, formation of the direct-positive images mainly comprises the steps of subjecting a photographic material having an internal latent image silver halide emulsion layer to

(D) 35 imagewise exposure, and thereafter applying a treatment to form fog nuclei (hereinafter "fogging treatment") by a chemical action followed by surface development, or thereafter carrying out surface development while applying fogging treatment. Here, the fogging treatment can be carried out by use of a compound that forms fog nuclei (hereinafter "fogging agent").

(E) 40 Compounds of wide-ranging types can be used as the fogging agent used in the present invention, and this fogging agent may be satisfactory if it is present at the time of developing. For example, it may be contained in component layers other than a support of a light-sensitive material, preferably in silver halide emulsion layers in particular, or in a developing solution or a processing solution preceding the developing. It can also be used in an amount that may vary in a wide range depending on purposes, and may preferably be added in an amount of from 1 to 1,500mg, and preferably from 10 to 1,000 mg, per mol of silver halide when it is added in the silver

-continued  
(Examples of compounds)

(G)



5

(H)



10

15

20 The amount of this compound to be added in at least any one layer of the photographic component layers may preferably range from 0.001 to 0.50 g/m<sup>2</sup>, and more preferably from 0.005 to 0.20 g/m<sup>2</sup>. Also, the above compounds may be used alone or may be mixed by arbitrarily selecting two or more compounds. It is also possible to use a quinone derivative having not less than 5 carbon atoms by adding it to the compound represented by the above Formula (HA), so long as the effect of the present invention may not be impaired. In either case of these, the amount of the compound to be used even as a mixture may preferably range from 0.001 to 0.50 g/m<sup>2</sup>.

25 (B) The silver halide emulsion can be optically sensitized using sensitizing dyes commonly used. Combination of sensitizing dyes used in supersensitization of internal latent image silver halide emulsions, negative silver halide emulsions, etc. is also useful for the silver halide emulsion of the present invention. As to the sensitizing dyes, reference can be made on Research Disclosures No., 15162 and No. 17643.

(C) 30 In instances in which direct-positive images are obtained by using the direct-positive silver halide photographic light-sensitive material of the present invention, the direct positive images can be readily obtained by carrying out imagewise exposure (the so-called photography, i.e., exposing a light-sensitive material to light to form an image) according to a usual method, followed by surface development. More specifically, formation of the direct-positive images mainly comprises the steps of subjecting a photographic material having an internal latent image silver halide emulsion layer to

(D) 35 imagewise exposure, and thereafter applying a treatment to form fog nuclei (hereinafter "fogging treatment") by a chemical action followed by surface development, or thereafter carrying out surface development while applying fogging treatment. Here, the fogging treatment can be carried out by use of a compound that forms fog nuclei (hereinafter "fogging agent").

(E) 40 Compounds of wide-ranging types can be used as the fogging agent used in the present invention, and this fogging agent may be satisfactory if it is present at the time of developing. For example, it may be contained in component layers other than a support of a light-sensitive material, preferably in silver halide emulsion layers in particular, or in a developing solution or a processing solution preceding the developing. It can also be used in an amount that may vary in a wide range depending on purposes, and may preferably be added in an amount of from 1 to 1,500mg, and preferably from 10 to 1,000 mg, per mol of silver halide when it is added in the silver

halide emulsion layers. When it is added in the processing solution such as the developing solution, it may also be added in an amount of from 0.01 to 5 g/l, and particularly preferably from 0.05 to 1 g/l.

The fogging agent used in the present invention includes compounds having a group that adsorbs on a silver halide surface, as exemplified by hydrazines, as described in U.S. Pat. Nos. 2,563,785 and 2,588,982, or hydrazides or hydrazine compounds, as described in U.S. Pat. No. 3,227,552; salts of heterocyclic quaternary nitrogen compounds, as described in U.S. Pat. Nos. 3,615,615, 3,718,470, 3,719,494, 3,734,738 and 3,759,901; and also acylhydrazinophenylthio ureas, as described in U.S. Pat. No. 4,030925. These fogging agents can also be used in combination. For example, Research Disclosure No 15162 discloses that a non-adsorptive fogging agent is used in combination with an adsorptive fogging agent.

As the fogging agent used in the present invention, either adsorptive ones or non-adsorptive ones can be used, and they can also be used in combination.

To set out useful examples of the fogging agent, they include hydrazine compounds such as hydrazine hydrochloride, phenylhydrazine hydrochloride, 4-methyl-phenylhydrazine hydrochloride 1-formyl-2-(4-methyl-phenyl)hydrazine, 1-acetyl-2-phenylhydrazine, 1-acetyl-2-(4-acetamidophenyl)hydrazine, 1-methylsulfonyl-2-phenylhydrazine, 1-benzoyl-2-phenylhydrazine, 1-methylsulfonyl-2-(3-phenylsulfonamidophenyl)hydrazine, and formaldehyde phenylhydrazine; N-substituted quaternary cycloammonium salts such as 3-(2-formylethyl)-2-methylbenzothiazolium bromide, 3-(2-formylethyl)-2-propylbenzothiazolium bromide, 3-(2-acetylethyl)-2-benzylbenzoselenazolium bromide, 3-(2-acetylethyl)-2-benzyl-5-phenyl-benzoxazolium bromide, 2-methyl-3-[3-(phenylhydrazono)propyl]benzothiazolium bromide, 2-methyl-3-[3-(p-tolylhydrazono)propyl]benzothiazolium bromide 2-methyl-3-[3 (p-sulfophenylhydrazono)propyl]benzothiazolium bromide, 2-methyl-3-[3-(p-sulfophenylhydrazono)pentyl]benzothiazolium iodide, 1,2-dihydro-3-methyl-4-phenylpyrido[2,1-b]benzothiazolium bromide, 1,2-dihydro-3-methyl-4-phenylpyrido[2,1-b]-5-phenylbenzoxazolium bromide, 4,4'-ethylene-bis(1,2-dihydro-3-methylpyrido[2,1-b]benzothiazolium bromide, and 1,2-dihydro-3-methyl-4-phenylpyrido[2,1-b]benzoselenazolium bromide; 5-[(1-ethylnaphtho(1,2-b)thiazolin-2-ylideneethylidene]-1-(2-phenylcarbazoyl)methyl-3-(4-sulfamoylphenyl)-2-thiohydantoin, 5-(3-ethyl-2-benzothiazolinylidene)-3-[4-(2-formylhydrozino)phenyl]rhodanine, 1-[4-(2-formylhydrazino)phenyl]-3-phenylthiourea, and 1,3-bis [4-(2-formylhydrazino)phenyl]thiourea.

The direct-positive silver halide photographic light-sensitive material of the present invention is subjected to developing in the presence of the fogging agent after imagewise exposure to light to form the direct-positive image. Any desired developing is employed as the developing method of the direct-positive light-sensitive material according to the present invention, but preferably a surface developing method may be used. This surface developing method is meant by the processing carried out with use of a developing solution substantially containing no silver halide solvent.

Developing agents that can be used in the developing solution used in the development of the direct-positive light sensitive material according to the present invention include commonly available silver halide developing agents, as exemplified by polyhydroxybenzenes

such as hydroquinone, aminophenols, 3-pyrazolidones, ascorbic acid and derivatives thereof, reductones, phenylenediamines, or a mixture of any of these. They specifically include hydroquinone, aminophenol, N-methylaminophenol, 1-phenyl-3-pyrazolidone, 1-phenyl-4,4-dimethyl-3-pyrazolidone, 1-phenyl-4-methyl-4-hydroxymethyl-3-pyrazolidone, ascorbic acid, N,N-diethyl-p-phenylenediamine, diethylamino-o-toluidine, 4-amino-3-methyl-N-ethyl-N-( $\beta$ -methanesulfonamidoethyl)aniline, and 4-amino-3-methyl-N-ethyl-N-( $\beta$ -hydroxyethyl)aniline. These developing agents can be previously contained in emulsions so that they may act on silver halide during immersion in an aqueous high-pH solution.

The developing solution used in the present invention may further contain a specific antifogging agent and a development restrainer, or it is also possible to optionally incorporate these developing solution additives into component layers of the light-sensitive material. Usually useful antifogging agents include heterocyclic thiones or aromatic and aliphatic mercapto compounds such as benzotriazoles, as exemplified by 5-methylbenzotriazole, benzoimidazoles, benzothiazoles, benzoxazoles, and 1-phenyl-5-meroaptotetrazole. The developing solution may also contain a development accelerator as exemplified by polyalkylene oxide derivatives or quaternary ammonium salt compounds.

In the direct-positive light-sensitive material also, it is common, after developing of the silver halide light-sensitive material in general, to carry out fixing or bleach-fixing, such that fixing is carried out with use of a processing solution containing a silver halide solvent, in order to remove unnecessary silver halide, or, in instances in which color images are obtained by developing, bleach-fixing is carried out with use of a processing solution containing a silver halide solvent and an oxidant, in order to remove unnecessary silver halide and metallic silver formed by development. In instances where photographic light-sensitive materials on which, after developing, the fixing or bleach-fixing can be directly carried out through no washing or no stopping using an acidic bath are used to make rapid the processing, the minimum density of an image can be small suppressed and thus an image with good quality can be obtained.

It is a matter of option to add various photographic additives in the emulsion containing the silver halide grains according to the present invention.

Other additives that are used in the present invention depending on purposes are wetting agents including, for example, dihydroxyalkane film property improving agents suitably including, for example, water-dispersible finely particulate polymeric materials obtained by emulsion polymerization, such as a copolymer of alkyl acrylate or alkyl methacrylate with acrylic acid or methacrylic acid, a styrene/maleic acid copolymer, and a styrene/maleic anhydride/half alkyl ester copolymer; coating aids including saponin, and polyethylene glycol lauryl ether. It is also a matter of option to use other photographic additives including gelatin plasticizers, surface active agents, ultraviolet absorbents, pH adjusters, antioxidants, antistatic agents, thickening agents, graininess improving agents, dyes, mordants, brightening agents, development speed regulators, and matting agents.

The silver halide emulsions prepared as described above are coated on a support optionally interposing subbing layers, halation-preventive layers and filter

layers, to obtain the internal latent image silver halide photographic light-sensitive material.

It is useful to apply the direct-positive silver halide photographic light-sensitive material according to the present invention in color photography. In this instance, cyan, magenta and yellow dye image-forming couplers may preferably contained in the silver halide emulsion. Those commonly used can be used as the couplers.

It is also useful to use ultraviolet absorbents as exemplified by thiazolidone, benzotriazole, acrylonitrile or benzophenone compounds to prevent the browning of dye images which is due to active light rays having short wavelengths, and particularly useful is to use alone or in combination Tinubin-PS, -320, -326, -327 and -328 (all available from Chiba-Geigy Corp.)

As the support, any desired supports can be used, but typical supports include polyethylene terephthalate film, polycarbonate film, polystyrene film, polypropylene film, cellulose acetate film, glass, baryta paper, and polyethylene-laminated paper, which have been optionally subjected to subbing.

In the emulsion containing the silver halide grains according to the present invention, gelatin, and besides, suitable gelatin derivatives can be used as protective colloids or binding materials depending on purposes. The present suitable gelatin derivatives may include, for example, acylated gelatin, guanidylated gelatin, carbamylated gelatin, cyanoethanolated gelatin, and esterified gelatin.

In the present invention, it is also possible to contain other hydrophilic binding material depending on purposes, and suitable binding materials include gelatin, and besides, colloidal albumin, agar, gum arabic, dextran, alginic acid, cellulose derivatives such as cellulose acetate having been hydrolyzed to an acetyl content of 19% to 20%, polyacrylamide, imidized polyacrylamide, casein, vinyl alcohol polymers containing a urethane carboxylic acid group or cyanoacetyl group, such as vinyl alcohol/vinyl aminoacetate copolymer; polyvinyl alcohol, polyvinyl pyrrolidone, hydrolyzed polyvinyl acetate, polymers obtained by polymerization of a protein or saturated acylated protein with a monomer having a vinyl group, polyvinylpyridine, polyvinylamine, polyaminoethyl methacrylate, and polyethyleneamine, which can be added to photographic component layers such as emulsion layers, intermediate layers, protective layers, filter layers and backing layers depending on purposes. A suitable plasticizer, lubricant or the like can be further contained in the above hydrophilic binders depending on purposes.

The component layers of the direct-positive light-sensitive material according to the present invention can be hardened using any desired suitable hardening agents. These hardening agents include chromium salts, zirconium compounds, and aldehyde (for example, formaldehyde or mucohalogen acid), halotriazine polyepoxy, compound, ethyleneimine, vinylsulfone or acryloyl hardening agents.

It is also possible for the photographic light-sensitive material according to the present invention to be provided on its support with a number of various photographic component layers such as emulsion layers, filter layers, intermediate layers, protective layers, subbing layers, backing layers, and halation preventive layers.

## EXAMPLES

The present invention will be described below in a specific manner by giving Examples, but is by no means limited to these.

### EXAMPLE 1

#### (Preparation of Em-1)

A monodisperse silver chlorobromide emulsion Em-1 was prepared in the following manner.

While controlling to 40° C. an aqueous solution containing (i) a seed emulsion comprising ossein gelatin and silver bromide of 0.11  $\mu\text{m}$  in average grain size and (ii) ammonia, an aqueous solution containing ammonia and silver nitrate and an aqueous solution containing potassium bromide were simultaneously added in the first-mentioned solution according to a controlled double jet method to obtain silver bromide core grains having an average grain size of 0.15  $\mu\text{m}$ . The rate of addition at this time was made to be a rate of 70% of the maximum addition rate at which any new silver halides are not produced. In that occasion, the pH and pAg of the emulsion in the course of addition were so controlled that grains having a grain form of a cube can be obtained, using an aqueous solution containing potassium bromide and an aqueous solution containing acetic acid.

To the resulting silver bromide emulsion of 0.15  $\mu\text{m}$ , an aqueous solution containing ammonia and silver nitrate and an aqueous solution containing potassium bromide and sodium chloride (KBr:NaCl=50:50 in molar ratio) were further simultaneously added according to the controlled double jet method, and shells were formed until the average grain size came to be 0.215  $\mu\text{m}$ . The rate of addition at this time was made to be a rate of 50% of the maximum addition rate at which any new silver halides are not produced. In that occasion, the pH and pAg of the emulsion in the course of addition were so controlled that grains having a cubic grain form can be obtained, using an aqueous solution containing potassium bromide and sodium chloride (KBr:NaCl=50:50 in molar ratio) and an aqueous solution containing acetic acid. Subsequently, washing was carried out to remove water-soluble salts, followed by addition of gelatin, thus making the emulsion Em-1. Electron-microscopic observation confirmed that this emulsion had a cubic grain form and a monodisperse emulsion having uniform grain size.

#### (Preparation of Em-2 to Em-7)

Monodisperse silver chlorobromide emulsions Em-2 to Em-7 were prepared in the same manner as the preparation of Em-1.

Provided that each emulsion was prepared under conditions described in Table 1 in regard to the grain size of seed emulsions, grain size of silver bromide core grains, and final grain size after formation of shells. Electron-microscopic observation confirmed that the resulting emulsions Em-2 to EM-7 had a cubic grain form and monodisperse emulsions having uniform grain size.

TABLE 1

|      | Average grain size ( $\mu\text{m}$ ) |                            |                  |
|------|--------------------------------------|----------------------------|------------------|
|      | Silver bromide seed emulsion         | Silver bromide core grains | Final grain size |
| Em-1 | 0.11                                 | 0.15                       | 0.215            |
| Em-2 | 0.11                                 | 0.18                       | 0.272            |
| Em-3 | 0.11                                 | 0.22                       | 0.329            |

TABLE 1-continued

|      | Average grain size ( $\mu\text{m}$ ) |                            |                  |
|------|--------------------------------------|----------------------------|------------------|
|      | Silver bromide seed emulsion         | Silver bromide core grains | Final grain size |
| Em-4 | 0.11                                 | 0.30                       | 0.443            |
| Em-5 | 0.26                                 | 0.41                       | 0.602            |
| Em-6 | 0.26                                 | 0.55                       | 0.817            |
| Em-7 | 0.26                                 | 0.75                       | 1.14             |

## (Preparation of Em-8)

A polydisperse silver chlorobromide emulsion Em-8 was prepared in the following manner.

While controlling to 60° C. an aqueous solution containing ossein gelatin and 0.75 mol of potassium bromide, an aqueous solution containing 0.7 mol of silver nitrate was added over a period of 40 minutes to obtain polydisperse silver bromide. Subsequently, in the solution containing the polydisperse silver bromide, an aqueous solution containing 0.53 mol of sodium chloride and 0.32 mol of potassium bromide and an aqueous solution containing 0.8 mol of silver nitrate were simultaneously added over a period of 20 minutes. After the addition was completed, washing was carried out to remove water-soluble salts, followed by addition of gelatin, thus making the emulsion Em-8 (average grain size: 0.33  $\mu\text{m}$ ).

Electron-microscopic observation confirmed that this emulsion is a polydisperse silver chlorobromide emulsion. Also this emulsion is a polydisperse emulsion having one broad peak in the grain size distribution curve.

Next, sensitizing dye shown below as GD-1 was added in emulsions Em-1 to Em-8 to obtain green-sensitive emulsions Em-1 to Em-8.

Using the resulting green-sensitive emulsions Em-1 to Em-8, Sample No. 1 was prepared in the following way.

On a double-sided polyethylene laminate paper, a first layer to an eighth layer were provided by coating as shown in Table 2. SA-1 and SA-2 were used as coating aids, and HA-1 and HA-2 were used as hardening agents to carry out the coating.

TABLE 2

|                                                                         | Sample No. 1:<br>(Numerals indicate coating weight; unit: mg/dm <sup>2</sup> ) |
|-------------------------------------------------------------------------|--------------------------------------------------------------------------------|
| <u>Sixth layer (ultraviolet-absorbing layer)</u>                        |                                                                                |
| Ultraviolet absorbent (UV-1)                                            | 0.65                                                                           |
| Ultraviolet absorbent (UV-2)                                            | 1.95                                                                           |
| Solvent (SO-3)                                                          | 1.0                                                                            |
| Gelatin                                                                 | 7.8                                                                            |
| Colloidal silica                                                        | 0.07                                                                           |
| <u>Fifth layer (blue-sensitive emulsion layer)</u>                      |                                                                                |
| Silver chlorobromide emulsion (average grain size: 0.88 $\mu\text{m}$ ) | 4.4*                                                                           |

TABLE 2-continued

|                                                                                      | Sample No. 1:<br>(Numerals indicate coating weight; unit: mg/dm <sup>2</sup> ) |
|--------------------------------------------------------------------------------------|--------------------------------------------------------------------------------|
| Silver chlorobromide emulsion (average grain size: 0.44 $\mu\text{m}$ )              | 1.2*                                                                           |
| Blue-sensitive sensitizing dye (BD-1)                                                |                                                                                |
| Fogging agent (FA-1)                                                                 | 5.5 $\times 10^{-5}$ mol/mol Ag                                                |
| Yellow coupler (YC-1)                                                                | 8.2                                                                            |
| Image stabilizer (AO-3)                                                              | 3.0                                                                            |
| Anti-stain agent (AS-1)                                                              | 0.25                                                                           |
| Anti-stain agent (AS-2)                                                              | 0.25                                                                           |
| Solvent (SO-1)                                                                       | 5.2                                                                            |
| Gelatin                                                                              | 14.3                                                                           |
| <u>Fourth layer (yellow colloidal layer)</u>                                         |                                                                                |
| Yellow colloidal silver                                                              | 1.05                                                                           |
| Color-mixing preventive agent (AS-1)                                                 | 0.40                                                                           |
| Solvent (SO-2)                                                                       | 0.49                                                                           |
| Polyvinyl pyrrolidone                                                                | 0.47                                                                           |
| Gelatin                                                                              | 4.2                                                                            |
| <u>Third layer (green-sensitive emulsion layer)</u>                                  |                                                                                |
| Silver bromide emulsion (Em-2)                                                       | 1.30*                                                                          |
| Silver bromide emulsion (Em-4)                                                       | 2.00*                                                                          |
| Green-sensitive sensitizing dye (GD-1)                                               |                                                                                |
| Fogging agent (FA-1)                                                                 | 5.5 $\times 10^{-5}$ mol/mol Ag                                                |
| Magenta coupler (MC-1)                                                               | 2.4                                                                            |
| Image stabilizer (AO-1)                                                              | 2.2                                                                            |
| Image stabilizer (AO-2)                                                              | 1.55                                                                           |
| Anti-stain agent (AS-1)                                                              | 0.03                                                                           |
| Anti-stain agent (AS-2)                                                              | 0.19                                                                           |
| Solvent (SO-4)                                                                       | 3.15                                                                           |
| Anti-irradiation dye (AI-1)                                                          | 0.13                                                                           |
| Gelatin                                                                              | 13.0                                                                           |
| <u>Second layer (intermediate layer)</u>                                             |                                                                                |
| Color-mixing preventive agent (AS-1)                                                 | 0.55                                                                           |
| Solvent (SO-2)                                                                       | 0.72                                                                           |
| Gelatin                                                                              | 7.5                                                                            |
| <u>First layer (red-sensitive emulsion layer)</u>                                    |                                                                                |
| Silver chlorobromide emulsion (average grain size: 0.62 $\mu\text{m}$ )              | 2.08*                                                                          |
| Silver chlorobromide emulsion (average grain size: 0.22 $\mu\text{m}$ )              | 0.70*                                                                          |
| Silver chlorobromide emulsion (average grain size: 0.20 $\mu\text{m}$ )              | 0.50*                                                                          |
| Red-sensitive sensitizing dye (RD-1), (RD-2)                                         |                                                                                |
| Fogging agent (FA-1)                                                                 | 5.5 $\times 10^{-5}$ mol/mol Ag                                                |
| Cyan coupler (CC-1)                                                                  | 2.08                                                                           |
| Cyan coupler (CC-2)                                                                  | 2.08                                                                           |
| Image stabilizer (AO-3)                                                              | 2.2                                                                            |
| Anti-stain agent (AS-2)                                                              | 0.15                                                                           |
| Solvent (SO-1)                                                                       | 3.3                                                                            |
| Anti-irradiation dye (AI-2)                                                          | 0.09                                                                           |
| Gelatin                                                                              | 13.8                                                                           |
| <u>Support</u>                                                                       |                                                                                |
| Paper support laminated with polyethylene on its both sides; thickness: Back coating | 140 $\mu\text{m}$                                                              |
| Gelatin                                                                              | 53                                                                             |
| Colloidal silica                                                                     | 6.0                                                                            |

\*Coating weight is in terms of silver.

RD-1



-continued



4,943,518

**45****46**

-continued

MC-2



YC-1



SO-1



SO-2



SO-3



SO-4



AS-1



AS-2



AO-1

4,943,518

47



48

-continued

AO-2



AO-3

HA-1



HA-2



UV-1



UV-2



SA-1



SA-2



AI-1



-continued



Samples No. 2 to No. 10 were prepared in the same manner as Sample No. 1.

Provided that in the composition of the third layer (green-sensitive emulsion layer) in Sample No. 1, emulsions and magenta couplers were varied as shown in Table 3.

Further, Sample No. 11 was prepared in the same manner as Sample No. 1, except that Third layer-A and Third layer-B were provided in place of Third layer. Compositions of Third layer-A and Third layer-B were as follows:

|                                 | Third layer-B          | Third layer-A          |
|---------------------------------|------------------------|------------------------|
| Silver chlorobromide emulsion   | Em-4 2.00*             | Em-2 1.30*             |
| Green-sensitizing dye           | GD-1                   | GD-1                   |
| Fogging agent (EA-1) mol/mol Ag | 5.5 × 10 <sup>-5</sup> | 5.5 × 10 <sup>-5</sup> |
| Magenta coupler (No. 10)        | 1.44                   | 0.96                   |
| Image stabilizer (AO-1)         | 1.32                   | 0.88                   |
| Image stabilizer (AO-2)         | 0.75                   | 0.50                   |
| Anti-stain agent (AS-1)         | 0.018                  | 0.012                  |
| Anti-stain agent (AS-2)         | 0.114                  | 0.076                  |
| Solvent SO-4                    | 0.078                  | 0.052                  |
| Gelatin                         | 7.8                    | 5.2                    |

TABLE 3

| Sample No. | Emulsion                 | Magenta coupler    | Remarks |
|------------|--------------------------|--------------------|---------|
| 1          | Em-2 (1.30), Em-4 (2.00) | Comp. No. 10 (2.4) | Y       |
| 2          | Em-1 (1.30), Em-3 (2.00) | Comp. No. 46 (2.4) | Y       |
| 3          | Em-3 (1.30), Em-5 (2.00) | Comp. No. 10 (2.4) | X       |
| 4          | Em-4 (1.30), Em-6 (2.00) | Comp. No. 10 (2.4) | X       |
| 5          | Em-5 (1.30), Em-7 (2.00) | Comp. No. 10 (2.4) | X       |
| 6          | Em-2 (1.30), Em-5 (2.00) | Comp. No. 10 (2.4) | Y       |
| 7          | Em-1 (0.65), Em-2 (0.65) | Comp. No. 10 (2.4) | Y       |
|            | Em-4 (2.00)              |                    |         |
| 8          | Em-1 (0.65), Em-2 (0.65) | Comp. No. 22 (2.4) | Y       |
|            | Em-5 (2.00)              |                    |         |
| 9          | Em-8                     | Comp. No. 10 (2.4) | X       |
| 10         | Em-2 (1.50), Em-4 (2.30) | MC-2 (2.9)         | X       |
| 11         | Em-2 (1.30), Em-4 (2.00) | Comp. No. 10 (2.4) | Y       |

Y: Present invention; X: Comparative example

The numerals in parentheses indicate coating weight, mg/dm<sup>2</sup>, which is in terms of silver in the case of emulsions.

The resulting respective samples were exposed to light through an optical wedge with use of a sensitometer, and then processed according to the processing steps shown below.

| (Processing 1)   |                         |              |
|------------------|-------------------------|--------------|
| Processing steps | Time                    | Temperature  |
| Color developing | 2 min. 30 sec.          | 33° C.       |
| Bleach-fixing    | 40 sec.                 | 33° C.       |
| Stabilizing      | 20 sec.,<br>three times | 33° C.       |
| Drying           | 30 sec.                 | 60 to 80° C. |

| (Color developing solution 1)      |       |        |
|------------------------------------|-------|--------|
| Diethylenetriaminepentaacetic acid | 2.0 g |        |
| Benzyl alcohol                     |       | 12.8 g |

| -continued |                                                                                                |
|------------|------------------------------------------------------------------------------------------------|
| 20         | Diethylene glycol 3.4 g                                                                        |
|            | Sodium sulfite 2.0 g                                                                           |
|            | potassium bromide 0.5 g                                                                        |
|            | Hydroxylamine sulfate 2.6 g                                                                    |
|            | Sodium chloride 3.2 g                                                                          |
|            | 3-methyl-4-amino-N-ethyl-N-( $\beta$ -methanesulfonamidoethyl)aniline 4.25 g                   |
| 25         | Potassium carbonate 30.0 g                                                                     |
|            | Brightening agent (a 4,4'diaminostilbenedisulfonic acid derivative) 1.0 g                      |
|            | Made up by adding water, to 1 1                                                                |
|            | pH 10.5                                                                                        |
| 30         | The pH was adjusted using potassium hydroxide and sulfuric acid.                               |
|            | <u>(Bleach-fixing solution)</u>                                                                |
|            | Ammonium thiosulfate (54 wt. %) 150 cc                                                         |
|            | Sodium sulfite 15 g                                                                            |
|            | Ferric (III) ammonium ethylenediaminetetraacetate 55 g                                         |
| 35         | Sodium ethylenediaminetetraacetate (dihydrate) 4 g                                             |
|            | Glacial acetic acid 8.61 g                                                                     |
|            | Made up by adding water, to 1 1                                                                |
|            | pH 5.4                                                                                         |
|            | The pH was adjusted using ammonia water or hydrochloric acid.                                  |
| 40         | <u>(Stabilizing solution)</u>                                                                  |
|            | 1-Hydroxyethylidene-1,1-diphosphonic acid (60%) 1.6 ml                                         |
|            | Bismuth chloride 0.35 g                                                                        |
|            | Polyvinyl pyrrolidone 0.25 g                                                                   |
|            | Ammonia water 2.5 ml                                                                           |
| 45         | Trisodium nitrilotriacetate 1.0 g                                                              |
|            | 5-Chloro-2-methyl-4-isothiazolin-3-one 50 mg                                                   |
|            | 2-Octyl-4-isothiazolin-3-one 50 mg                                                             |
|            | Brightening agent (4,4'diaminostilbene type) 1.0 g                                             |
|            | Made up by adding water, to 1 1                                                                |
|            | pH 7.5                                                                                         |
| 50         | (The pH was adjusted using potassium hydroxide or hydrochloric acid.)                          |
|            | <u>(Processing 2)</u>                                                                          |
|            | Same as Processing 1 except that the pH of the color developing solution was adjusted to 10.8. |
|            | <u>(Processing 3)</u>                                                                          |
| 55         | Same as Processing 1 except that the pH of the color developing solution was adjusted to 11.2. |

Sensitometry was carried out on the resulting images, and the maximum density, straight line portion gamma, and straight line portion gamma/toe gamma were evaluated only about magenta images. Results obtained are shown in Table 4. Here, the toe gamma is indicated by an absolute value of the slope of the straight line portion connecting a density point of minimum density +0.15 and a density point of minimum density +0.5 in the characteristic curve. Also, the straight line portion gamma/toe gamma was evaluated as an index that shows the linearity of the characteristic curve.

TABLE 4

| Sample No. | Processing | Maximum density | Straight line portion gamma | Straight line portion gamma/toe gamma |
|------------|------------|-----------------|-----------------------------|---------------------------------------|
| 1 (Y)      | 1          | 2.12            | 1.35                        | 1.12                                  |
|            | 2          | 2.20            | 1.36                        | 1.21                                  |
|            | 3          | 2.22            | 1.38                        | 1.23                                  |
| 2 (Y)      | 1          | 2.13            | 1.43                        | 1.10                                  |
|            | 2          | 2.18            | 1.46                        | 1.16                                  |
|            | 3          | 2.19            | 1.47                        | 1.23                                  |
| 3 (X)      | 1          | 1.96            | 1.16                        | 1.05                                  |
|            | 2          | 2.04            | 1.31                        | 1.15                                  |
|            | 3          | 2.11            | 1.45                        | 1.33                                  |
| 4 (X)      | 1          | 1.83            | 1.25                        | 1.03                                  |
|            | 2          | 1.92            | 1.40                        | 1.14                                  |
|            | 3          | 2.01            | 1.45                        | 1.23                                  |
| 5 (X)      | 1          | 1.73            | 1.27                        | 1.01                                  |
|            | 2          | 1.92            | 1.39                        | 1.16                                  |
|            | 3          | 1.98            | 1.46                        | 1.21                                  |
| 6 (Y)      | 1          | 2.17            | 1.32                        | 1.14                                  |
|            | 2          | 2.21            | 1.37                        | 1.20                                  |
|            | 3          | 2.22            | 1.42                        | 1.19                                  |
| 7 (Y)      | 1          | 2.31            | 1.40                        | 1.15                                  |
|            | 2          | 2.33            | 1.37                        | 1.18                                  |
|            | 3          | 2.35            | 1.42                        | 1.21                                  |
| 8 (Y)      | 1          | 2.30            | 1.36                        | 1.15                                  |
|            | 2          | 2.30            | 1.40                        | 1.21                                  |
|            | 3          | 2.31            | 1.42                        | 1.23                                  |
| 9 (X)      | 1          | 2.13            | 1.26                        | 0.92                                  |
|            | 2          | 2.19            | 1.45                        | 1.17                                  |
|            | 3          | 2.15            | 1.50                        | 1.29                                  |
| 10 (X)     | 1          | 2.00            | 1.29                        | 1.06                                  |
|            | 2          | 2.06            | 1.29                        | 1.17                                  |
|            | 3          | 2.11            | 1.42                        | 1.26                                  |
| 11 (Y)     | 1          | 2.10            | 1.32                        | 1.10                                  |
|            | 2          | 2.17            | 1.32                        | 1.14                                  |
|            | 3          | 2.18            | 1.34                        | 1.16                                  |

(Y): Present invention; (X): Comparative example

As will be evident from the results shown in Table 4, the samples No. 1, No. 2, No. 6, No. 7, No. 8 and No. 11 of the present invention show a higher maximum density, a sufficiently high maximum density even with variation of the pH of the color developing solution, and a stabilities in the straight line portion gamma/toe gamma ratio serving as an index that indicates the variation of the straight line portion gamma and the linearity of the characteristic curve.

## EXAMPLE 2

## (Preparation of Em-9)

A monodisperse silver chlorobromide emulsion Em-9 was prepared in the following manner. In a core emulsion comprising ossein gelatin and cubic silver chlorobromide ( $\text{AgBr:AgCl}=50:50$  in molar ratio) of  $0.15 \mu\text{m}$  in average grain size, sodium thiosulfate and sodium chloroaurate were added to effect chemical sensitization, and thereafter two kinds of aqueous solutions, an aqueous solution of silver nitrate and an aqueous solution containing potassium bromide and sodium chloride ( $\text{KBr:NaCl}=50:50$  in molar ratio), were simultaneously added according to the controlled double jet method to obtain a cubic core/shell emulsion of  $0.25 \mu\text{m}$  in average grain size. In the resulting emulsion, sodium thiosulfate and sodium chloroaurate were further added to effect chemical sensitization of the surfaces to an appropriate degree, thus obtaining an internal latent image core/shell emulsion Em-9.

## (Preparation of Em-10)

Em-0 was prepared in the same manner as Em-9. Provided that a cubic silver chlorobromide emulsion of  $0.32 \mu\text{m}$  was used as the core emulsion in place of the cubic silver chlorobromide emulsion of  $0.15 \mu\text{m}$ , and

also the covering with shells was so carried out that the core/shell emulsion may have an average grain size of  $0.47 \mu\text{m}$ . In both emulsions, the silver halide composition of the core/shell emulsion was made to be  $\text{AgBr:AgCl}=50:50$  in molar ratio.

Using the resulting Em-9 and Em-10, samples No. 12 to No. 14 were prepared in the same manner as the sample No. 1 in the above Example 2.

Provided that, in the green-sensitive emulsion layer, the magenta coupler and fogging agent only were made different as shown in Table 5, from those of the sample No. 1, in addition to the employment of Em-9 and Em-10.

TABLE 5

| Sample No. | Emulsion                  | Magenta coupler | Fogging agent (mol/molAg)   |
|------------|---------------------------|-----------------|-----------------------------|
| 12         | Em-9 (1.50), Em-10 (2.20) | Compound No. 22 | FA-2 ( $4 \times 10^{-5}$ ) |
| 13         | Em-9 (1.50), Em-10 (2.20) | Compound No. 22 | FA-2 ( $6 \times 10^{-5}$ ) |
| 14         | Em-9 (1.50), Em-10 (2.20) | Compound No. 22 | FA-2 ( $1 \times 10^{-5}$ ) |



The resulting samples were subjected to the processing (Processing 1) in Example 1 using the color developing solution 1. They were also subjected to Processings 2 to 6, respectively, which were carried out by replacing the color developing solution 1 with color developing solutions 2 to 6 obtained by changing the composition in the color developing solution 1 only in respect of what are shown in Table 6.

TABLE 6

| Color developing solution No. | Composition         |                             |
|-------------------------------|---------------------|-----------------------------|
|                               | Potassium carbonate | Hydroxylamine nitrate       |
| 1                             | 30 g                | 2.6 g                       |
| 2                             | 30 g                | —                           |
| 3                             | 30 g                | Diethylhydroxylamine 2.4 g  |
| 4                             | 9 ml                | Hydroxylamine nitrate 2.6 g |
| 5                             | 9 ml                | —                           |
| 6                             | 9 ml                | Diethylhydroxylamine 2.4 g  |

Sensitometry was carried out on the resulting and the maximum density and minimum density were measured only in respect of magenta images to obtain the results shown in Table 7.

TABLE 7

| Color developing solution No. | Sample No. | Maximum density | Minimum density |
|-------------------------------|------------|-----------------|-----------------|
| 1                             | 12         | 1.75            | 0.16            |
|                               | 13         | 2.09            | 0.18            |
|                               | 14         | 2.17            | 0.22            |
| 2                             | 12         | 1.98            | 0.14            |

TABLE 7-continued

| Color developing solution No. | Sample No. | Maximum density | Minimum density |
|-------------------------------|------------|-----------------|-----------------|
| 3                             | 13         | 2.10            | 0.16            |
|                               | 14         | 2.13            | 0.17            |
| 4                             | 12         | 2.08            | 0.14            |
|                               | 13         | 2.20            | 0.15            |
| 5                             | 14         | 2.22            | 0.16            |
|                               | 12         | 1.97            | 0.14            |
| 6                             | 13         | 2.21            | 0.17            |
|                               | 14         | 2.24            | 0.19            |
| 10                            | 12         | 2.25            | 0.15            |
|                               | 13         | 2.33            | 0.15            |
| 15                            | 14         | 2.37            | 0.16            |
|                               | 12         | 2.29            | 0.13            |
| 20                            | 13         | 2.36            | 0.14            |
|                               | 14         | 2.38            | 0.15            |

The results shown in Table 7 tell that better photographic performances can be obtained when the phosphoric acid compound is used in the color developing solution and no hydroxylamine is contained in the color developing solution.

What is claimed is:

1. A direct positive silver halide photographic light-sensitive material which comprises a support having thereon a blue-sensitive emulsion layer containing a yellow color coupler, at least one green-sensitive emulsion layer and a red-sensitive emulsion layer containing a cyan color coupler and, is capable of forming a positive image by developing with a color developer in the presence of a fogging agent after exposure to light, wherein the green-sensitive emulsion comprises silver halide grains having at least two peaks on the size distribution curve thereof, where the grain size corresponding to the smallest grain size peak among said at least two peaks is not more than 0.3  $\mu\text{m}$ ; and at least one of the magenta coupler represented by the following Formula (M-1);



Formula (M-1)

wherein Z represents a group of non-metal atoms necessary to complete a nitrogen-containing heterocyclic ring which may have a substituent; X represents a hydrogen atom or a group capable of being split off upon reaction with the oxidized product of a color developing agent; and R represents a hydrogen atom or a substituent.

2. The material of claim 1, wherein said silver halide grains contained in said green sensitive emulsion layer have two peaks on the size distribution curve thereof.
3. The material of claim 1, wherein said silver halide grains contained in said green-sensitive emulsion layer have three peaks on the size distribution curve thereof.
4. The material of claim 1, wherein said grain size corresponding to the smallest grain size peak is within the range of from 0.05  $\mu\text{m}$  to 0.3  $\mu\text{m}$ .
5. The material of claim 1, wherein grain size at the peaks other than the smallest grain size peak is not more than 1.5  $\mu\text{m}$ .

6. The material of claim 5, wherein grain size at the peaks other than the smallest grain size peak is not more than 1.0  $\mu\text{m}$ .

7. The material of claim 6, wherein grain size at the peaks other than the smallest grain size peak is not more than 0.7  $\mu\text{m}$ .

8. The material of claim 1, wherein difference of said peaks in grain size is not more than 10% based on a grain size corresponding to greater grain size peak.

9. The material of claim 1, wherein said green-sensitive emulsion layer comprises a plurality of emulsion layers each containing emulsions each of which has a single peak at different grain size from each other on the grain size distribution curve thereof.

10. The material of claim 1, wherein said green-sensitive emulsion layer comprises at least one layer of emulsion containing having at least two peaks on the grain size distribution curve thereof.

11. The material of claim 1, wherein said silver halide grains have core/shell structure.

12. The material of claim 1, wherein said silver halide grains are internal latent image type grains being not fogged on the surface thereof.

13. The material of claim 1, wherein said substituent represented by R in Formula (M-1) is an alkyl group, an aryl group, an anilino group, an acylamino group, a sulfonamido group, an alkylthio group, an arylthio group, an alkenyl group, a cycloalkyl group, a halogen atom, a cycloalkenyl group, an alkinyl group, a heterocyclic group, a sulfonyl group, a sulfinyl group, an acyl group, a carbamoyl group, a sulfamoyl group, a cyano group, an alkoxy group, an aryloxy group, a heterocyclic oxy group, a siloxy group, an acyloxy group, a carbamoyloxy group, an amino group, an alkylamino group, an imido group, a ureido group, a sulfamoylaminogroup, an alkoxy carbonylaminogroup, an aryloxycarbonylaminogroup, a heterocyclic thio group, a spyro compound residue or a bridged hydrocarbon compound residue.

14. The material of claim 1, wherein said group represented by the X in Formula (M-1) is a halogen atom, an alkoxy group, an aryloxy group, a heterocyclic oxy group, an acyloxy group, a sulfonyloxy group, an alkoxycarbonyloxy group, an aryloxycarbonyl group, an alkyloxalyloxy group, an alkoxyoxalyloxy group, an alkylthio group, an arylthio group, a heterocyclic thio group, an alkyloxythiocarbonyloxy group, an acylamino group, a sulfonamido group, a nitrogen-containing heterocyclic ring combined through N atom, an alkyloxycarbonylaminogroup, an aryloxycarbonylaminogroup, a carboxyl group or a group of

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915



wherein R<sub>1</sub> to R<sub>8</sub> and X are the same as R and X in Formula (M-I), respectively.

16. The material of claim 15, wherein said coupler is represented by the following Formula (M-VIII);



wherein R<sub>1</sub>, X and Z are the same as R, X and Z in Formula (M-I), respectively.

17. The material of claim 16, wherein said coupler is represented by Formula (M-II) or (M-III).

18. The material of claim 17, wherein said coupler is represented by Formula (M-II).

19. The material of claim 1, wherein said coupler is contained in said green-sensitive emulsion layer in an amount of from  $1 \times 10^{-3}$  to 1 mole per mole of silver halide.

20. The material of claim 1, wherein said material comprises said fogging agent.

21. The material of claim 20, wherein said fogging agent is contained in an amount of from 1 mg to 1500 mg per mole of silver halide.

22. A method for forming a direct positive image comprising

a step for imagewise exposing to light a silver halide photographic light-sensitive material which comprises a support having thereon a blue-sensitive emulsion layer containing a yellow color coupler, at least one green-sensitive emulsion layer and a red-sensitive emulsion layer containing a cyan color coupler, and

(M-II)

5

(M-III)

10

(M-IV)

15

(M-V)

20

(M-VI)

25

(M-VII)

30

Formula (M-VIII)

40

a step for developing said silver halide photographic light-sensitive material with a color developer in the presence of a fogging agent, wherein the green-sensitive emulsion comprises silver halide grains having at least two peaks on the size distribution curve thereof, where the grain size corresponding to the smallest grain size peak among said at least two peaks is not more than 0.3  $\mu\text{m}$ ; and at least one of the magenta coupler represented by the following Formula (M-1);

Formula (M-I)



wherein Z represents a group of non-metal atoms necessary to complete a nitrogen-containing heterocyclic ring which may have a substituent; X represents a hydrogen atom or a group capable of being split off upon reaction with the oxidized product of a color developing agent; and R represents a hydrogen atom or a substituent.

23. The method of claim 22, wherein said developer contains a phosphoric acid compound.

24. The method of claim 23, wherein said phosphoric acid compound is a compound represented by the following Formula (P-I), (P-II) or (P-III)

)  $\text{A}^1 \text{mP}_m \text{O}_{3m}$

Formula (P-I)

$\text{A}^2, \text{A}^3, \text{A}^4 \text{nP}_n \text{O}_{3n+1}$

Formula (P-II)

$\text{A}^5, \text{A}^6, \text{A}^7 \text{PO}_3$

Formula (P-III)

wherein  $\text{A}^1$  to  $\text{A}^7$  each represent a hydrogen atom, an alkali metal atom or an alkyl group; m and n each represent an integer of from 1 to 20.

25. The method of claim 24, wherein said phosphoric acid compound is a compound represented by the following Formula (P-IV), (P-V), (P-VI), (P-VII), (P-VIII), (P-IX), (P-X) or (P-XI);

$\text{M}_m \text{P}_m \text{O}_{3m}$

Formula (P-IV)

$\text{M}_{n+2} \text{P}_n \text{O}_{3n+1}$

Formula (P-V)

wherein M represents an alkali metal atom; m and n each represent an integer of from 1 to 20;

$\text{B}_1-\text{R}_{21}-\text{Z}-\text{R}_{22}-\text{COOH}$

Formula (P-IV)



Formula (P-VII)

wherein E represents a substituted or unsubstituted alkylene group, a cycloalkylene group, a phenylene group, a  $-\text{R}_{27}-$  group, a  $-\text{OR}_{27}-$  group, a  $-\text{R}_{27}-\text{OR}_{27}-\text{R}_{27}-$  group or a  $-\text{R}_{27}\text{ZR}_{27}-$  group; Z represents  $=\text{NR}_{27}-\text{B}_6$  or  $=\text{NB}_6$ ; R<sub>21</sub> to R<sub>27</sub> each represent a substituted or unsubstituted alkylene group; B<sub>1</sub> to B<sub>6</sub> each represent a hydrogen atom, a  $-\text{OH}$  group, a  $-\text{COOM}$  group, a  $-\text{PO}_3\text{M}_2$  group, where at least one of B<sub>1</sub> and B<sub>6</sub> represents  $-\text{PO}_3\text{M}_2$  group, at least one of B<sub>2</sub> to B<sub>5</sub> represents  $-\text{PO}_3\text{M}_2$  group.

group; and M represents a hydrogen atom or an alkali metal atom;



Formula (P-VIII)

wherein  $R_{28}$  represents a lower alkyl group, an aralkyl group, a nitrogen-containing 6-membered ring group; M represents a hydrogen atom or an alkali metal atom;



Formula (P-IX)

wherein  $R_{29}$  to  $R_{31}$  each represent a hydrogen atom, a  $-OH$  group, a lower alkyl group;  $C_1$  to  $C_3$  each represent a hydrogen atom, a  $-OH$  group, a  $-COOH$  group,  $-PO_3M_3$  group, or  $Nj_2$  group; where  $j$  represents a hydrogen atom, a lower alkyl group, a  $-C_2H_4OH$  group or a  $-PO_3M_2$  group; M represents a hydrogen atom or an alkali meta atom; and n and m each represent 0 or 1;



Formula (P-X)

wherein  $R_{32}$  and  $R_{33}$  each represent a hydrogen atom, an alkyl group having 1 to 12 carbon atoms, an alkenyl group, a cyclic alkyl group; and M represents a hydrogen atom or an alkali metal atom;



Formula (P-XI)

wherein  $R_{34}$  represents an alkyl group having 1 to 12 carbon atoms, an alkoxy group having 1 to 12 carbon atoms, a monoalkylamino group having 1 to 12 carbon atoms, a dialkylamino group having 1 to 12 carbon atoms, an amino group, an aryloxy group having 1 to 24 carbon atoms, an arylamino group having 6 to 24 carbon atoms or an amyoxy group;  $Q_1$  to  $Q_3$  each represent a  $-OH$  group, an alkoxy group, having 1 to 24 carbon atoms, an aralkyloxy group, an aryloxy group,  $-OM$  group, where M is a cation, an amino group, a morpholino group, a cyclic amino group, an alkylamino group, a dialkylamino group, an arylamino group or an alkyloxy group.

26. The method of claim 23, wherein said phosphoric acid compound is contained in said color developer in an amount of 3 to 200 g/l.

27. The method of claim 22, wherein said color developer substantially not contains hydroxyamine.

28. The method of claim 22, wherein said color developer contains a hydroxylamine derivative represented by the following Formula (HA);



Formula (HA)

wherein  $R_{41}$  and  $R_{42}$  each represent a hydrogen atom or an alkyl group provided that both of  $R_{41}$  and  $R_2$  are not hydrogen atom in the same time;  $R_{41}$  and  $R_{42}$  may be combined to form a ring.

5 29. The method of claim 28, said hydroxylamine derivative is contained in said color developer in an amount of from 0.2 to 50 g/l.

30. The method of claim 22, said color developer contains said fogging agent.

10 31. The method of claim 30, said fogging agent is contained in said color developer in an amount of from 0.5 g/l to 30 g/l.

15 32. The method of claim 22, wherein said silver halide grains contained in said green sensitive emulsion layer have two peaks on the size distribution curve thereof.

33. The method of claim 22, wherein said silver halide grains contained in said green-sensitive emulsion layer have three peaks on the size distribution curve thereof.

20 34. The method of claim 22, wherein said grain size corresponding to the smallest grain size peak is within the range of from 0.05  $\mu m$  to 0.3  $\mu m$ .

35. The method of claim 22, wherein grain size at the peak other than the smallest grain size peak is not more than 1.5  $\mu m$ .

25 36. The method of claim 35, wherein grain size at the peak other than the smallest grain size peak is not more than 1.0  $\mu m$ .

37. The method of claim 36, wherein grain size at the peak other than the smallest grain size peak is not more than 0.7  $\mu m$ .

38. The method of claim 22, wherein difference of said peaks in grain size is not more than 10 % based on a grain size corresponding to greater grain size peak.

39. The method of claim 22, wherein said green-sensitive emulsion layer comprises a plurality of emulsion layers each containing emulsions each of which has a single peak at different grain size from each other on the grain size distribution curve thereof.

40. The method of claim 22, wherein said green-sensitive emulsion layer comprises at least one layer containing an emulsion having at least two peaks on the grain size distribution curve thereof.

41. The method of claim 22, wherein said silver halide grains have core/shell structure.

42. The method of claim 22, wherein said silver halide grains are internal latent image type grains being not fogged on the surface thereof.

43. The method of claim 22, wherein said substituent represented by R in Formula (M-1) is an alkyl group, an aryl group, an anilino group, an acylamino group, a sulfonamido group, an alkylthio group, an arylthio group, an alkenyl group, a cycloalkyl group, a halogen atom, a cycloalkenyl group, an alkynyl group, a heterocyclic group, a sulfonyl group, a sulfinyl group, an acyl group, a carbamoyl group, a sulfamoyl group, a cyano group, an alkoxy group, an aryloxy group, a heterocyclic oxy group, a siloxy group, an acyloxy group, a carbamoyloxy group, an amino group, an alkylamino group, an imido group, a ureido group, a sulfamoyl amino group, an alkoxy carbonyl amino group, an aryloxy carbonyl amino group, a heterocyclic thio group, a spiro compound residue or a bridged hydrocarbon compound residue.

44. The method of claim 22, wherein said group represented by the X in Formula (M-1) is a halogen atom, an alkoxy group, an aroxy group, a heterocyclic oxy group, an acyloxy group, a sulfonyloxy group, an alkoxy carbonyloxy group, an aryloxy carbonyl group, an

alkyloxalyloxy group, an alkoxyoxalyloxy group, an alkylthio group, an arylthio group, a heterocyclic thio group, an alkyloxythiocarbonyloxy group, an acylamino group, a sulfonamido group, a nitrogen-containing heterocyclic ring combined through N atom, an alkyloxycarbonylamino group, an aryloxycarbonylamino group, a carboxyl group or a group of



wherein R<sub>1</sub>' and Z' are each the same as R and Z in Formula 1 and R<sub>2</sub>' and R<sub>3</sub>' are each a hydrogen atom, an alkyl group, an aryl group or a heterocyclic group.

45. The method of claim 22, wherein said coupler is represented by the following Formula (M-II), (M-III), (M-IV), (M-V), (M-VI) or (VII);



(M-II)

30 wherein R<sub>1</sub>, X and Z are the same as R, X and Z in Formula I, respectively.

46. The method of claim 22, wherein said coupler is represented by Formula (M-II) or (M-III);

(M-III)

47. The method of claim 46, wherein said coupler is represented by Formula (M-II) or (M-III).

48. The method of claim 47, wherein said coupler is represented by Formula (M-II).

49. The method of claim 22, wherein said coupler is contained in said green-sensitive emulsion layer in an amount of from  $1 \times 10^{-3}$  to 1 mole per mole of silver halide.

50. The method of claim 22, wherein said silver halide photographic light sensitive material comprises said fogging agent.

51. The method of claim 50, wherein said fogging agent is contained in an amount of from 1 mg to 1500 mg per mole of silver halide.

45

50

55

60

65

-continued

(M-V)



(M-VI)



(M-VII)



10

15

20

25

30

35

40

45

Formula (M-VIII)

wherein R<sub>1</sub>, X and Z are the same as R, X and Z in Formula I, respectively.

46. The method of claim 22, wherein said coupler is represented by Formula (M-II) or (M-III).

47. The method of claim 46, wherein said coupler is represented by Formula (M-II) or (M-III).

48. The method of claim 47, wherein said coupler is represented by Formula (M-II).

49. The method of claim 22, wherein said coupler is contained in said green-sensitive emulsion layer in an amount of from  $1 \times 10^{-3}$  to 1 mole per mole of silver halide.

50. The method of claim 22, wherein said silver halide photographic light sensitive material comprises said fogging agent.

\* \* \* \* \*